

1

**3,140,210**  
**BINDER SYSTEM FOR PROPELLANTS AND**  
**EXPLOSIVES**

Henry T. Sampson, Urbana, Ill., assignor to the United States of America as represented by the Secretary of the Navy  
 No Drawing. Filed Jan. 25, 1963, Ser. No. 254,822  
 4 Claims. (Cl. 149—88)  
 (Granted under Title 35, U.S. Code (1952), sec. 266)

The invention described herein may be manufactured and used by or for the Government of the United States of America for governmental purposes without the payment of any royalties thereon or therefor.

The present invention relates to improved binder compositions and the preparation thereof. More specifically, it relates to an improved binder system for plastic-bonded explosives and composite propellants.

In the fields concerned with compressible explosives and cast composite propellants it has been found that most of the binder materials in use have high initial viscosity so that a high percentage of solid ingredients cannot be combined or worked in and the product remain compressible or castable. Most of the binders being used today, including polyurethanes, polysulfides, and nitrocellulose plastisols, require high curing temperatures in order to achieve the desired physical properties.

The general purpose of this invention is to provide a binder system for composite propellants and cast explosives which embraces all the advantages of similarly employed binder systems and possesses none of the aforementioned disadvantages.

An object of the present invention is the provision of a binder composition which is compatible with a large number of high energy ingredients used in explosives and propellants.

Another object is the provision of a low viscosity binder composition which permits high loading of propellant and explosive ingredients.

A further object of the invention is the provision of a binder system which will give increased energy to explosive and propellant compositions.

Still another object is to provide a binder system which has good adhesive properties.

Other objects, features and many of the attendant advantages of this invention will be readily appreciated as the same become better understood by reference to the following detailed description.

Broadly, this invention contemplates a basic binder composition comprising about 30 to 40% by weight castor oil (CasO), about 11 to 15% by weight dipropylene glycol (DPG), about 20 to 30% by weight 2,4-tolylene diisocyanate (TDI) and about 15 to 35% by weight trimethylol ethane trinitrate (TMETN).

The binder composition is prepared by mixing castor oil, dipropylene glycol and tolylene diisocyanate in a reaction flask for about twenty minutes at 32° F. This reaction is highly exothermic and the viscosity of the reactants can be controlled by keeping the temperature below 120° F. Since a by-product of the reaction is carbon dioxide, the reaction must be carried out under vacuum if a bubble-free product is desired. However, it is possible to mix under normal pressure and degas the product after mixing. The trimethylol ethane trinitrate is added

2

after the mixing step. At this point the binder composition is ready to be mixed with explosive or propellant ingredients and cast into a suitable container (rocket motor, warhead). To obtain maximum physical properties, the polymer should be cured for five days at 120° F. Shorter curing times if desired may be obtained by increasing the curing temperature or by adding a catalyst such as ferric acetyl acetone in an amount not exceeding one part per 50 parts of polymer.

10 The three binder compositions listed in Table I below with their corresponding physical properties are illustrative of the present invention.

*Table I*

| Example  | Ingredients (Percent by weight) |      |      |       | Tensile Strength (p.s.i.) | Elongation (Percent) |
|----------|---------------------------------|------|------|-------|---------------------------|----------------------|
|          | CasO                            | DPG  | TDI  | TMETN |                           |                      |
| I-----   | 36.0                            | 13.0 | 26.5 | 24.5  | 270                       | 290                  |
| II-----  | 31.9                            | 11.6 | 23.5 | 33.0  | 110                       | 200                  |
| III----- | 39.1                            | 14.2 | 28.8 | 17.9  | 665                       | 260                  |
| IV-----  | 32.5                            | 11.7 | 22.4 | 33.4  | 117                       | 191                  |

CasO—Castor oil.

DPG—Dipropylene glycol.

TDI—2,4-tolylene diisocyanate.

TMETN—Trimethylol ethane trinitrate.

The approximate curing time for the above formulations was five days at 140° F.

This binder is a polyurethane type polymer. Apparently the hydroxyl groups on glycol and castor oil react with the isocyanate groups to form a urethane bond, and the trimethylol ethane trinitrate functions as an external plasticizer.

35 Table II below shows the results of progress to determine the curing conditions which give the best binder physical properties using the formulation set out in Example IV above.

*Table II*

| Sample (Example IV) | Cure Time (days) | Cure Temp. (° F.) | Hardness (Shore Sclerometer) | Tensile Strength (p.s.i.) | Elongation (Percent) |
|---------------------|------------------|-------------------|------------------------------|---------------------------|----------------------|
| 1-----              | 2                | 120               | 19.4                         | 55.0                      | 254                  |
| 4-----              | 2                | 140               | 23.0                         | 96.3                      | 240                  |
| 5-----              | 2                | 160               | 38.6                         | 131.0                     | 137                  |
| 6-----              | 4                | 120               | 40.8                         | 106.4                     | 195                  |
| 7-----              | 4                | 140               | 43.4                         | 117.0                     | 191                  |
| 8-----              | 4                | 160               | 52.2                         | 147.0                     | 155                  |

50 This data shows that after two days, the 140° F. curing temperature produces the best binder.

The basic binder formulation may be modified by increasing or decreasing the percent of trimethylol ethane trinitrate (TMETN). For example, the binder with no TMETN has a strength of 2500 p.s.i. and 150% elongation; the binder with 30% TMETN has a tensile strength of 200 p.s.i. and an elongation of 200%. Furthermore, other nitrated plasticizers such as diethylene glycol dinitrate, 1,4-butanediol dinitrate, polyglycidal nitrate, and pentaerythritol trinitrate may be substituted for trimethylol ethane trinitrate.

All or part of the dipropylene glycol may be replaced with polypropylene glycol.

Obviously many modifications and variations of the

present invention are possible in the light of the above teachings. It is therefore to be understood that within the scope of the appended claims the invention may be practiced otherwise than as specifically described.

What is claimed is:

1. A binder composition comprising the following ingredients:

| Ingredients:                                                                                                                                               | Percent by weight |
|------------------------------------------------------------------------------------------------------------------------------------------------------------|-------------------|
| Castor oil.....                                                                                                                                            | 30 to 40          |
| Dipropylene glycol.....                                                                                                                                    | 11 to 15          |
| 2,4-tolylene diisocyanate.....                                                                                                                             | 20 to 30          |
| Trimethylol ethane trinitrate.....                                                                                                                         | 15 to 35          |
| 2. The composition of claim 1 wherein a mixture of equal amounts of dipropylene glycol and polypropylene glycol are used in lieu of dipropylene glycol. 15 |                   |

3. A binder composition consisting essentially of the following ingredients:

| Ingredients:                       | Percent by weight |
|------------------------------------|-------------------|
| Castor oil.....                    | 32.5              |
| Dipropylene glycol.....            | 11.7              |
| 2,4-tolylene diisocyanate.....     | 22.4              |
| Trimethylol ethane trinitrate..... | 33.4              |

4. A binder composition consisting essentially of the following ingredients:

| Ingredients:                       | Percent by weight |
|------------------------------------|-------------------|
| Castor oil.....                    | 36.0              |
| Polypropylene glycol.....          | 13.0              |
| 2,4-tolylene diisocyanate.....     | 26.5              |
| Trimethylol ethane trinitrate..... | 24.5              |

No references cited.